

## UNITED STATES PATENT OFFICE

2,182,045

## PROCESS OF WATERPROOFING FIBROUS MATERIAL

Edward B. Bell, Lowell, Mass., assignor to Hall Laboratories, Inc., Pittsburgh, Pa., a corporation of Pennsylvania

No Drawing. Application July 12, 1937,  
Serial No. 153,293

10 Claims. (Cl. 149—6)

This invention relates to a process of waterproofing fibrous material, and more particularly to a process of waterproofing leather.

The invention is applicable to the waterproofing of vegetable or animal fibers which in their raw or in their manufactured condition have the disadvantage of absorbing moisture. By the present invention, such materials may be made substantially impervious to water with freedom 10 from shrinking, cracking or change of color. The invention is particularly applicable to waterproofing leather fibers and will be described as applied to the treatment of leather, it being understood, however, that it may be employed in 15 treating other animal or vegetable fibrous material. Leather is especially susceptible to harm by contact with water, resulting in cracking and shrinking of the leather. It also causes loss of color and strength in the leather.

20 The following is a specific example of a process of waterproofing leather according to the present invention. The leather to be waterproofed is immersed in a solution of sodium hexametaphosphate, alum, soap and ammonia at a temperature 25 of approximately 120° F. After soaking for a short time, the leather is removed and dried preferably at moderate temperature. For waterproofing 5 grams of leather the following quantities of alum, sodium oleate, sodium hexameta- 30 phosphate and ammonia may be dissolved in 50 ml. of water:

|                          | Grams |
|--------------------------|-------|
| Alum                     | 0.053 |
| Sodium oleate            | 2.750 |
| Sodium hexametaphosphate | 2.500 |
| Ammonia                  | 2.500 |

The leather is soaked in this bath for several minutes at a temperature of 120° F., the solution 40 squeezed out, and the leather dried at a moderate temperature. The drying temperature should not be above that which will harm the leather and may be any temperature higher than that which will cause evaporation of the ammonia. As a result of this treatment, the leather 45 is waterproofed without affecting its color, feel, odor or strength of the fiber.

The alum and sodium oleate react to form 50 aluminum soap which is kept in solution by the combination of the ammonia and the sodium hexametaphosphate. The leather which has been soaked in this solution, upon drying, liberates the ammonia which causes the deposition of aluminum soap throughout the fibers of the 55 leather.

Instead of employing alum, I may use salts of other metals, such as lead or tin or other amphoteric metals which do not form complexes with the ammonia or with other solvents which may be employed in place of ammonia. The preferred metal used in forming the metallic soap is aluminum.

In place of ammonia, I may use other alkaline materials which are solvents for metallic soaps and which evaporate at temperatures which will 10 not harm the leather or other fibrous material which is being waterproofed. Examples of such other alkaline solvents for metallic soaps are triethanolamine or diethanolamine.

In place of sodium oleate, I may employ any 15 other suitable fatty acid soap.

I may employ other phosphates instead of sodium hexametaphosphate, commonly known as "Graham's salt". I may employ the alkali-metal pyrophosphates or tripolyphosphates, for example sodium pyrophosphate ( $Na_4P_2O_7$ ) or sodium tripolyphosphate ( $Na_5P_3O_{10}$ ). The alkali-metal metaphosphates, tripolyphosphates and pyrophosphates may be considered as "molecularly dehydrated phosphates" since they may be 20 formed from alkali-metal orthophosphates by dehydrating the orthophosphates so as to effect an atomic re-arrangement within the phosphate molecule. These molecularly dehydrated phosphates may be considered as derived from phosphoric acid containing less water than orthophosphoric acid. The term "molecularly dehydrated alkali-metal phosphate" as used in the claims is intended to include the alkali-metal metaphosphates, tripolyphosphates or pyrophosphates. 30 Any of these phosphates may be employed in 35 conjunction with the ammonia or other solvent for dissolving the metallic soap.

Textile fibers, such for example as wool, silk, cotton or linen, or paper fibers may be treated 40 either before or after fabrication with the waterproofing solution and the solvent evaporated to impregnate the fibers with the metallic soap.

The invention is not limited to the example 45 given or to the specific materials mentioned, but may be otherwise embodied or practiced within the scope of the following claims.

I claim:

1. A process of waterproofing fibrous material, 50 which comprises treating it with a solution of a salt of an amphoteric metal, a water-soluble soap, an alkaline solvent for the metallic soap, said solvent evaporating at a temperature which will not harm the material being treated, and a 55

- molecularly dehydrated alkali-metal phosphate, and evaporating the solvent to deposit the metallic soap.
2. A process of waterproofing fibrous material, which comprises treating it with a solution of a salt of an amphoteric metal, a water-soluble soap, ammonia and a molecularly dehydrated alkali metal phosphate, and evaporating the ammonia to deposit the metallic soap.
- 10 3. A process of waterproofing fibrous material, which comprises treating it with a solution of a salt of an amphoteric metal, a water-soluble soap, ammonia and an alkali-metal metaphosphate, and evaporating the solvent to deposit the metallic soap.
- 15 4. A process of waterproofing fibrous material, which comprises treating it with a solution of a salt of an amphoteric metal, a water-soluble soap, ammonia, and Graham's salt, and evaporating the solvent to deposit the metallic soap.
5. A process of waterproofing fibrous material, which comprises treating it with a solution of a salt of an amphoteric metal, a water-soluble soap, ammonia and an alkali-metal pyrophosphate, and evaporating the solvent to deposit the metallic soap.
- 20 6. A process of waterproofing fibrous material, which comprises treating it with a solution of a salt of an amphoteric metal, a water-soluble soap, ammonia and an alkali-metal tripolyphosphate, and evaporating the solvent to deposit the metallic soap.
- 25 7. A process of waterproofing fibrous material, which comprises treating it with a solution of an aluminum salt, a water-soluble soap, ammonia and a molecularly dehydrated alkali-metal phosphate, and evaporating the ammonia to deposit the metallic soap.
- 10 8. A process of waterproofing leather, which comprises treating it with a solution of a salt of an amphoteric metal, a water-soluble soap, ammonia and a molecularly dehydrated alkali-metal phosphate, and evaporating the ammonia to deposit the metallic soap.
- 15 9. A process of waterproofing leather, which comprises treating it with a solution of an aluminum salt, a water-soluble soap, ammonia and a molecularly dehydrated alkali-metal phosphate, and evaporating the ammonia to deposit the metallic soap.
- 20 10. A process of waterproofing leather, which comprises treating it with a solution of alum, water-soluble soap, ammonia and a molecularly dehydrated alkali-metal phosphate, and evaporating the ammonia to deposit the metallic soap.

EDWARD B. BELL.